

F. SAVAGE.

METHOD OF MANUFACTURING TONE ARMS FOR TALKING MACHINES AND THE LIKE.  
APPLICATION FILED DEC. 28, 1918.

1,313,559.

Patented Aug. 19, 1919.

Fig. 1.



Fig. 2.

Inventor  
Frederick Savage,  
by his attorneys

Edward M. Wight

# UNITED STATES PATENT OFFICE.

FREDERICK SAVAGE, OF LONDON, ENGLAND.

METHOD OF MANUFACTURING TONE-ARMS FOR TALKING-MACHINES AND THE LIKE.

1,813,559.

Specification of Letters Patent.

Patented Aug. 13, 1919.

Application filed December 23, 1916. Serial No. 332,731.

To all whom it may concern:

Be it known that I, FREDERICK SAVAGE, a subject of the King of Great Britain, residing at 31 Severn's road, London, England, have invented a new and useful Improved Method of Manufacturing Tone-Arms for Talking-Machines and the like, of which the following is a specification.

In the accompanying drawings:—

10 Figure 1 is a side elevation of a tone arm constructed in accordance with my invention.

Fig. 2 is a plan view showing the two sections of the tone arm before they are joined.

15 My method of manufacturing tone arms for talking machines and the like consists in taking sheets of paper, cardboard, felt, strawboard, or any suitable woven cotton fiber or the like and cutting them into 20 blanks which can be molded into the shapes and sizes of the tone arm desired.

I then dampen the blanks and press them into molds of two opposite longitudinal halves of the tone arm.

25 An alternative method is to mold the two halves of the tone arm in paper or wood pulp. When the two halves prepared in either of these ways are dry, I sprinkle powdered resin in the hollow or inner side and burn in the same with hot iron or press. The two halves are then placed together and fastened with hot melted size or the like. Any suitable size which does not absorb 30 moisture may be employed. The ordinary size prepared from animal glue is found most efficient. A hollow tone arm is thus formed, lined with resin. I then add strips of paper, cardboard, felt, strawboard, or 35 suitable woven cotton fiber or the like, binding the said strips around the tone arm, or placing them lengthwise, fastening them together with hot melted size, until the re-

quired substance or thickness is obtained. The tone arm is then dried and smoothed, coated with chilled size and finished, being colored, varnished, or painted with metallic paints and the like as may be desired.

Suitable fittings are then added for attaching the tone arm to the carrier end for attaching the sound box to the tone arm.

A non-metallic tone arm thus prepared has many advantages; it has no metallic sound or affinity for notes of sound entering into the music such as are caused by vibration in the metal tone arm attached to talking machines of present make, and resulting in distortion and impure notes. The burning of the resin into the inner surface of the arm gives clearness and brilliancy to the music, while the strips of sized paper give a 50 membranous formation, preventing any after sound and consequently acting as a damper, as in a piano, to all notes played.

In Fig. 2 of the drawing I have shown the two sections A, B of the tone arm made in the manner before described. The two longitudinal sections are brought together and united as before explained, their interiors treated with melted resin, and strip material C is wound around the two sections 70 in the manner indicated. In Fig. 1 one end of the strip material is shown as free, but this end is fastened down in obvious ways.

What I claim is:—

The method of manufacturing tone arms 75 of non-metallic material which consists in molding non-metallic substances in sections, fastening together the sections, treating their interior with melted resin, and winding the whole externally with strip material. 80

In testimony that I claim the foregoing as my invention I have signed my name this 13th day of December, A. D. 1916.

FREDERICK SAVAGE